

1

3,007,783

## MOTOR FUEL COMPOSITIONS

William S. Young, Albert C. Condo, Jr., James B. Hunter, and Hyman Iserson, Newtown Square, Pa., assignors of one-half to The Atlantic Refining Company, Philadelphia, Pa., a corporation of Pennsylvania, and of one-half to Pennsalt Chemicals Corporation, Philadelphia, Pa., a corporation of Pennsylvania  
No Drawing. Filed Nov. 18, 1958, Ser. No. 774,596  
4 Claims. (Cl. 44—69)

This invention relates to improved motor fuels which will provide a reduced octane requirement increase and inhibit surface ignition in internal combustion engines. The invention more specifically relates to motor fuels in the gasoline boiling range containing an organofluoro phosphorus compound.

In recent years there have been developed internal combustion engines for use in motor cars which because of their high compression ratio require fuels of exceedingly high octane number. In order to produce such fuels economically it has been found necessary to add to the gasoline tetraethyl lead antiknock fluid in amounts ranging up to 3 cc. per gallon of gasoline. Moderately high octane number fuels have been found to satisfy the octane requirements of the engines while the engines are new but as the engines are used they require increasingly higher octane number fuels with the result that after a few months of operation only the very highest octane number fuels can be used in them.

This increase in octane requirement that an engine may experience during the whole or any part of its operating life is termed "octane number requirement increase" and is usually abbreviated to ORI. ORI has been found to be caused by combustion chamber deposits, which deposits it is believed increase the octane requirement of the engine for at least two reasons. The deposits decrease the physical volume of the combustion chamber and thus in effect increase the compression ratio of the engine which in turn raises the octane number requirement of the engine. The deposits also have a heat insulating effect which reduces the rate of heat transfer from the combustion chamber to the cooling system. This causes excessive heat to be transferred to the incoming air-fuel mixture which sensitizes the mixture and promotes autoignition. Thus as the engine is operated the amount of deposits increases and the octane number requirement increases. Moreover, it has been suggested also that these deposits produce hot spots in the combustion chamber where preignition can occur; that is, the hot, incandescent spot in the combustion chamber will cause the explosion of the gasoline-air mixture instead of the explosion being caused by the firing of the spark plug. This ignition generally occurs prior to the firing of the spark plug and hence this phenomenon is often termed preignition or surface-ignition. Preignition or surface-ignition often produces an effect similar to that of the "knocking" of low octane number fuels in a high octane requirement situation.

Heretofore gasoline additives have been devised which when used with fuels containing tetraethyl lead provide a reduction in the formation of combustion chamber deposits within the engine. Other additives have been devised which when added to a fuel containing tetraethyl lead inhibit surface ignition or preignition phenomena.

A motor fuel composition now has been found, however, which simultaneously will reduce the formation of combustion chamber deposits, thus preventing octane requirement increase of an engine and will also inhibit preignition or surface-ignition phenomena.

Accordingly it is an object of this invention to provide a motor fuel composition comprising a major

2

amount of hydrocarbons boiling in the gasoline range and a minor amount of an additive which is sufficient to reduce the octane requirement increase and inhibit surface-ignition in an internal combustion engine.

It is a further object of this invention to provide a motor fuel composition comprising a major amount of hydrocarbons boiling in the gasoline boiling range and a minor amount sufficient to reduce the octane requirement increase and inhibit surface-ignition in an internal combustion engine of a organofluoro phosphorus compound.

Further objects of this invention will be apparent from the description and claims that follow.

In accordance with the instant invention an organofluoro phosphorus compound is added to gasoline in minor amounts. These compounds are added preferably to a gasoline containing tetraethyl lead since the bulk of the gasoline presently being produced is leaded and it is the improvement of such fuels that is the primary purpose of this invention. The tetraethyl lead antiknock agent is employed in conventional amounts and contains the usual scavenging agents. In addition the gasoline may contain minor and conventional amounts of other additives such as solvent oils, gum inhibitors, dyes, lead stabilizers, carburetor anti-icing agents and similar additives.

The amount of organofluoro phosphorus compound which is added to the gasoline is preferably based on the amount of tetraethyl lead fluid contained in the gasoline and is expressed as a ratio between the gram atoms of phosphorus in the organofluoro phosphorus compound to the gram atoms of lead in the tetraethyl lead fluid in the gasoline. The preferred ratio ranges between 0.02 and 2 gram atoms of phosphorus to 3 gram atoms of lead. Since 3 cc. of tetraethyl lead fluid per gallon is equivalent to approximately 0.015 gram atom of lead per gallon the amount of phosphorus corresponding to the maximum amount of lead would range between 0.0001 and 0.01 gram atom of phosphorus per gallon of gasoline. The preferred ratio of phosphorus to lead, however, is between 0.2 and 1.0 gram atom of phosphorus to 3 gram atoms of lead, while the most preferred range is 0.3 to 0.5 gram atom of phosphorus to 3 gram atoms of lead.

The organofluoro phosphorus compounds suitable for use as gasoline additives in accordance with the instant invention have the general formula:



wherein  $R_1$ ,  $R_2$  and  $R_3$  are radicals selected from the group consisting of alkyl, aryl, alkaryl, aralkyl, fluoroalkyl, fluoro-alkaryl and fluoro-aralkyl radicals. The total number of carbon atoms in the molecule ranges between 3 and 30 and the total number of fluorine atoms in the molecule ranges between 2 and 15. In addition any carbon atom which is fluorine substituted bears at least two fluorine atoms and in the case of terminal carbon atoms the carbon may bear three fluorine atoms. In general, these compounds are prepared by reacting a fluoro-alcohol or a combination of an alcohol or phenol or substituted phenol and a fluoro-alcohol with phosphorus oxychloride.

The preferred compound for use in conjunction with the gasoline component of this invention is tris (trifluoroethyl) phosphate which has the following structural formula:



70

Other typical compounds included within the scope of this invention have structural formulas as follows:



The following examples will serve to illustrate the 25 preferred mode for carrying out the instant invention and to further define its scope and usefulness.

#### EXAMPLE I

Various fuel compositions were tested in a Briggs and Stratton, Model 5-S, single cylinder, air cooled, L-head internal combustion engine. The base gasoline employed was a commercial premium gasoline containing a blend of C<sub>4</sub> hydrocarbons, catalytically reformed naphtha and catalytically cracked naphtha together with isobutane-butylene alkylate. This gasoline had a boiling range of 90° F. to 420° F. and contained 3 cc. of conventional tetraethyl lead fluid per gallon. The lubricant employed was a conventional premium grade detergent-inhibitor additive lubricating oil of SAE 20 grade.

The engine was first run for 20 hours on the conventional gasoline fuel during which time the octane requirement of the engine increased from 62 to 71, i.e. an increase of 9 octane numbers. After the run the engine was dismantled and the interior surfaces of the combustion chamber and exhaust valve were cleaned of deposits. A new spark plug was used for each run.

After reassembly the engine was operated for a period of 20 hours on the same gasoline; however, in this run the gasoline contained tris (trifluoroethyl) phosphate in an amount corresponding to 1 gram atom of phosphorus per 3 gram atoms of lead in the lead tetraethyl and since the lead was at the 3 cc. level this amounted to 0.005 gram atom of phosphorus per gallon of gasoline. During this run the octane requirement of the engine increased only 2 numbers, i.e. from 62 to 64.

After disassembly, cleaning and reassembly the engine was operated for 20 hours on the same conventional gasoline which contained triethyl phosphate in an amount corresponding to 0.005 gram atom of phosphorus per

that where there are fluorine atoms in the latter compound there are hydrogen atoms in the former compound. During this run the octane requirement of the engine increased from 62 to 71, i.e. the same increase as found 5 for the blank run on the conventional fuel without additive.

The engine was again disassembled, cleaned, reassembled and run for 20 hours on the same conventional gasoline which however in this run contained tris (trifluoroethyl) phosphate in an amount corresponding to 0.4 gram atom of phosphorus per 3 gram atoms of lead, i.e. 0.002 gram atom of phosphorus per gallon of gasoline. The octane requirement of the engine increased from 62 to 63, an increase of only one number.

10 15 Each type of run was repeated a number of times in a randomized order with the ORI determined each time and with disassembly, cleaning and reassembly of the engine between each run. The results of these runs are set forth in Table I.

20

Table I

|                              | Additive | Blank fuel, no additive    | tris (trifluoroethyl) phosphate, 0.005 gram atoms of P per gallon | triethyl phosphate, 0.005 gram atoms of P per gallon | tris (trifluoroethyl) phosphate, 0.002 gram atoms of P per gallon |
|------------------------------|----------|----------------------------|-------------------------------------------------------------------|------------------------------------------------------|-------------------------------------------------------------------|
| Octane Requirement Increase. |          | 9<br>9<br>8<br>8<br>8<br>9 | 2<br>2<br>2<br>1                                                  | 9<br>8                                               | 1<br>2                                                            |
| Ave. ORI.....                |          | 8.5                        | 1.8                                                               | 8.33                                                 | 1                                                                 |

35 These data show that it is necessary to have the fluorine present in the compound to reduce ORI and that better results are obtained when the concentration level is at 0.002 gram atom of phosphorus per gallon than when it is above this amount. Additional tests have 40 demonstrated that if the ratio of phosphorus in the organofluoro phosphorus compound is below 0.02 gram atom to 3 gram atoms of lead in the form of lead tetraethyl in the gasoline this is not enough additive to provide the improvements desired according to the invention and correspondingly if the ratio of phosphorus to lead is in excess of 2 gram atoms of phosphorus to 3 gram atoms of lead no further improvement in engine 45 performance is noted.

50

#### EXAMPLE II

55 The same fuel and additive combinations employed in Example I, with the exception of the triethyl phosphate additive combination, were employed in a series of 100 hour runs in the same test engine used in Example I. The initial octane requirement of the engine was determined before the start of the test run and the octane requirement after each 20 hours of operation. The engine was not disassembled and cleaned until it had operated for the entire 100 hours. The results of 60 those tests are shown in Table II.

Table II

| Additive.....       | Blank fuel, No Additive |    |    |    |    |     | tris (trifluoroethyl) phosphate, 0.005 gram atoms of P per gallon |    |    |    |    | tris (trifluoroethyl) phosphate, 0.002 gram atoms of P per gallon |    |    |    |    |    |     |
|---------------------|-------------------------|----|----|----|----|-----|-------------------------------------------------------------------|----|----|----|----|-------------------------------------------------------------------|----|----|----|----|----|-----|
|                     | 0                       | 20 | 40 | 60 | 80 | 100 | 0                                                                 | 20 | 40 | 60 | 80 | 100                                                               | 0  | 20 | 40 | 60 | 80 | 100 |
| Time in Hours.....  |                         |    |    |    |    |     |                                                                   |    |    |    |    |                                                                   |    |    |    |    |    |     |
| Octane Requirement: |                         |    |    |    |    |     |                                                                   |    |    |    |    |                                                                   |    |    |    |    |    |     |
| Initial.....        | 56                      | 63 | 72 | 78 | 80 | 78  | 58                                                                | 61 | 68 | 74 | 75 | 75                                                                | 60 | 62 | 64 | 68 | 67 | 67  |
| Final.....          |                         | 7  | 16 | 22 | 24 | 22  | 3                                                                 | 10 | 16 | 17 | 17 | 17                                                                | 2  | 4  | 8  | 7  | 7  | 7   |
| ORI.....            |                         |    |    |    |    |     |                                                                   |    |    |    |    |                                                                   |    |    |    |    |    |     |

gallon of gasoline. The triethyl phosphate corresponds in structure to the tris (trifluoroethyl) phosphate except

75 These data show that the octane requirement of the engine increases to a equilibrium value with all fuels

and that if the additives of the instant invention are employed, the equilibrium value of the octane requirement of the engine is lower than that of a fuel not containing the additives of the invention.

## EXAMPLE III

In order to demonstrate the effectiveness of the fuels of this invention in providing reduced ORI and surface ignition under road test conditions several compositions of this invention were tested in a stock 1957 Oldsmobile 88 with a 9.5 to 1 compression ratio engine under normal city-suburban driving. After 1500 miles of operation using a commercial gasoline containing 3 cc. tetraethyl lead per gallon and a commercial organo phosphorus-containing additive without fluorine at the level of 0.002 gram atom of phosphorus per gallon of gasoline the octane requirement of the test engine was found to be 96.0.

After completely cleaning the engine of deposits and operating for 1500 miles on the same gasoline as above except that instead of the commercial phosphorus additive it contained 0.002 gram atom of phosphorus as tris (trifluoroethyl) phosphate the octane requirement was found to be 94.0.

The level of surface ignition of the engine also was found to be considerably lower when using the fuel containing the tris (trifluoroethyl) phosphate than when using fuel containing the same phosphorus level but without fluorine being present in the additive.

These tests demonstrated that the organofluoro phosphorus compounds of the instant invention are superior additives for providing reduced octane requirement increase and for inhibiting surface ignition as compared with additives which contain no fluorine and only an organo phosphorus compound.

We claim:

1. A gasoline motor fuel consisting essentially of hydrocarbons boiling in the gasoline range and containing tetraethyl lead antiknock agent together with an organofluoro phosphorus compound in an amount corresponding to from 0.02 to 2.0 gram atoms of phosphorus to 3 gram atoms of lead, the organofluoro phosphorus compound having the general formula:



5 wherein  $R_1$ ,  $R_2$  and  $R_3$  are radicals selected from the group consisting of alkyl, aryl, alkaryl, aralkyl, fluoroalkyl, fluoro-alkaryl and fluoro-aralkyl, the total number of carbon atoms in the molecule ranges between 3 and 30, the total number of fluorine atoms in the molecule 10 ranges between 2 and 15 and each fluorine substituted carbon atom has at least two fluorine atoms attached thereto.

15 2. A gasoline motor fuel consisting essentially of hydrocarbons boiling in the gasoline range and containing tetraethyl lead antiknock agent together with tris (trifluoroethyl) phosphate in an amount corresponding to from 0.02 to 2.0 gram atoms of phosphorus to 3 gram atoms of lead.

20 3. A gasoline motor fuel consisting essentially of hydrocarbons boiling in the gasoline range and containing tetraethyl lead antiknock agent together with tris (trifluoroethyl) phosphate in an amount corresponding to from 0.2 to 1.0 gram atom of phosphorus to 3 gram atoms of lead.

25 4. A gasoline motor fuel consisting essentially of hydrocarbons boiling in the gasoline range and containing tetraethyl lead antiknock agent together with tris (trifluoroethyl) phosphate in an amount corresponding to from 0.3 to 0.5 gram atom of phosphorus to 3 gram atoms of lead.

## References Cited in the file of this patent

## UNITED STATES PATENTS

|           |                             |               |
|-----------|-----------------------------|---------------|
| 2,833,635 | Hill et al. -----           | May 6, 1958   |
| 2,834,798 | Hechenbleikner et al. ----- | May 13, 1958  |
| 2,839,563 | Hechenbleikner -----        | June 17, 1958 |
| 2,892,691 | Howell -----                | June 30, 1959 |

## FOREIGN PATENTS

|           |                     |               |
|-----------|---------------------|---------------|
| 1,094,828 | France -----        | Dec. 15, 1954 |
| 1,100,185 | France -----        | Mar. 30, 1955 |
| 1,134,156 | France -----        | Nov. 26, 1956 |
| 683,405   | Great Britain ----- | Nov. 26, 1952 |

UNITED STATES PATENT OFFICE  
CERTIFICATION OF CORRECTION

Patent No. 3,007,783

November 7, 1961

William S. Young et al.

It is hereby certified that error appears in the above numbered patent requiring correction and that the said Letters Patent should read as corrected below.

Column 3, lines 3 to 6, the formula should appear as shown below instead of as in the patent:



same column 3, lines 7 to 10, the formula should appear as shown below instead of as in the patent:



same column 3, lines 17 to 20, the formula should appear as shown below instead of as in the patent:



Signed and sealed this 17th day of April 1962.

Attest:

ESTON G. JOHNSON  
Attesting Officer

DAVID L. LADD  
Commissioner of Patents